

## UNITED STATES PATENT OFFICE.

HUBERT A. MYERS, OF TOLEDO, AND ARTEEMES D. STRAW, OF WAUSEON, OHIO,  
ASSIGNORS TO THE HUBERT A. MYERS COMPANY, OF TOLEDO, OHIO, A CORPO-  
RATION OF OHIO.

## CONTAINER AND MOLD FOR MOLTEN METAL.

No Drawing. Original application filed January 27, 1921, Serial No. 440,501. Divided and this application filed January 18, 1922. Serial No. 529,030.

To all whom it may concern:

Be it known that we, HUBERT A. MYERS and ARTEEMES D. STRAW, citizens of the United States, and residents of Toledo, Lucas County, Ohio, and Wauseon, Fulton County, Ohio, respectively, have made an Invention Appertaining to Containers and Molds for Molten Metal; and we do hereby declare the following to be a full, clear, and exact description of the invention, such as will enable others skilled in the art to which it appertains to make and use the same.

This application is a division of our application, Sr. No. 440,501, filed January 27, 1921.

Our invention has for its object to provide articles or devices for manipulating molten metal, such as for containing or conveying or casting molten metal, and wherein in free flow or free delivery of the metal from the article may be obtained, either while the metal is in a molten, in a semi-plastic, or in a solid state. The invention particularly has for its object to produce articles for manipulating molten metals, such as runners, troughs, ladles, or molds, containing metal at or near the contact surfaces of the article with the molten metal, that are so constructed that erosion or pitting of the article by the metal will be avoided. When our invention is embodied in molds, rapid and economical production of smooth, perfect castings may be made without injury to the molds.

Heretofore unsuccessful efforts have been made to prevent the destructive action of molten metal on metal articles or articles containing metal at or near the contact surfaces of the article with the molten metal, by the use of coatings or linings formed of various materials, such as clay, graphite, and similar surfacing materials, since such coatings easily crack or are brushed from the permanent parts of the ladles or molds or pots, thus destroying their utility. Also some coating materials heretofore used cause pitting of the hot metal if it is allowed

to solidify within the article, and other materials will not adhere to the surface of the article if the heated metal is moved over the surface, and others will not withstand high temperatures.

Metal articles or metal containing articles for manipulating molten metal and embodying our invention are provided with a protective material that will not be removed or destroyed, or its efficiency injuriously affected, either by heat or from the contact and flow of the molten metal. The protective material also permits free delivery of the heated metal, and when the hot metal is allowed to solidify smooth surfaces are formed where contact is made with the articles, so that in case of molds, castings having smooth, perfectly formed surfaces can be made, whether the molds are cold or maintained at a relatively high temperature.

We treat or deposit on the surfaces of the article that come in contact with a molten metal, certain gasifiable or vapor-forming substances that will neutralize or prevent the injurious effects of the molten metal. If the gasifiable material is oxidizable in air at a temperature below the melting point of the metal manipulated or contained in the article, a coating of the oxide will also be formed over the article which will be heat insulating in character, and thus reduce the effect of the molten metal on the article and on the gas forming substance deposited at the surface of the article. We preferably use a material that will alloy with or have an affinity for or an ionic or electric attraction for the substances of which the body of the article is wholly or partially composed; or a material that will readily penetrate the surface of the article and thus impregnate the article; or a metalliferous gasifiable or vaporizing material that will deposit on or become incorporated within the surface of the article.

The gasifiable substance used is of such a character that it will gasify at a temperature below the melting point of the metal to be brought in contact with the article. In the

case of molds, the gasifying point of the gas forming substances should be above the temperature at which the mold is maintained in order to produce soft castings, and below the 5 temperature of the molten metal to be cast in the mold. The selection of the gas forming substances will therefore depend upon the melting point of the metal to be brought in contact with the article. For instance, if 0 molten brass is to be manipulated, gas forming substances having relatively low gasifying points should be used; such as cadmium and zinc chloride. In manipulating iron, materials such as zinc magnesium, cadmium 5 and barium may be used. If high speed steel is to be cast it may be found desirable to use zinc, barium or bismuth as a gas forming material, since these substances and compounds thereof, and mixtures containing 0 them, are gas or vapor forming substances, and produce a substantially perfect protective coating between the article and the metal. The term gas will be used herein to include both gas and vapor.

5 Zinc is especially suitable for use in protecting ferrous metal articles, or articles containing ferrous metals, from molten metals, particularly ferrous molten metals, for the reason that zinc has a vaporizing point 0 as well as a boiling point, that is, it has a gasifying point, below the melting point of iron, and thus will produce a small amount of gas substantially in film form between the article and the molten metal when subjected 5 to the heat of the molten metal. This will operate to protect the article and, if the metal is allowed to cool within the article, as in a mold, the metal contained in the article will be delivered with smooth surfaces and without pits or blow-holes. In case of a mold, some of the vapor or gas may be partially taken up by the mold or the casting, or both, and if any remains after the casting is discharged it will be precipitated 10 as white oxide of zinc on the surface of the mold. Also the zinc metal on its surface will be oxidized by contact with the air. Furthermore, the zinc has an affinity for and is electropositive to the iron and will automatically distribute itself under the action of the heat of the molten metal so as to keep the surfaces of the article supplied with the proper amount of zinc, and in case of molds, a sufficient quantity of the zinc will be drawn to the surface of the mold to form the required amount of gas at each casting operation without retreatment of the mold with zinc or its compounds. Moreover its gas is readily controlled by materials, such as lamp black, that may be readily deposited over the surface in the interim between casting operations. Thus in case of ferrous molds when used for casting ferrous metals, the molds may be heated and maintained at a substantially uniform tempera-

ture to produce soft castings and ejected, if desired, while the interior of the casting is still in a molten condition. Also ferrous castings may be made in ferrous molds without preheating, and the casting left in the 70 mold until it has hardened throughout. In any case, the casting and the mold are readily separated, which enables an assured delivery of all parts of the casting from the mold, even though some of the surfaces of the casting may be drawn over or parallel with the surface of the mold. Articles containing our invention thus may be used continuously or repeatedly without repeating the treatment or deposition of the protective material on their surfaces, and in the case of molds, repeated castings may be made without repeating the treatment, or, if desired, the molds may be quickly and easily treated after each casting or pouring 75 operation. Also castings may be easily discharged from the mold when they have set sufficiently to retain their form, or they may be permitted to remain in the mold as long as desired, whether the mold is hot or cold, and without injuriously affecting the matrix thereof or adhering to the mold.

When the articles have been properly treated with the protective material, only a small volume of gas will be formed from the gas forming material. If the gas forming substances are incorporated in the body of the article the heat from the molten metal will cause the formation of a limited amount of gas and will automatically and regulatively approach the heated surface of the article, and thus replenish the supply of such substances at the surface where it is needed. Also the oxide of the gas forming material, as in the case of zinc, will be produced when it comes in contact with the air, as upon removal of the molten metal from the article, or of a casting from a mold, if the article be a mold, and form a surface coating of metallic oxide on the article, which will tend to reduce the amount of the gas formed because of the heat resisting character of a finely divided oxide or of the gas confining character of an encrusted oxide. If the oxide is itself gasifiable it will generally only be so at a higher temperature than that at which the oxide is formed, and the amount of gas produced from the oxide will be comparatively small. If, on the other hand, the gas forming substance is located only on the molding surface the amounts of gas that are successfully formed may be controlled either by regulating the amount of the gas forming substances placed on the surface, or by depositing with it or upon it a suitable heat insulating material, such as lamp black, or oxide of a metal, such as zinc oxide.

We use preferably materials that will 130 alloy with or be absorbed or have an affinity

for the material of which the article is composed so that the gas forming substances may be readily incorporated in the article or will adhere thereto and thus insure a suitable supply of gas for continuous or repeated use of the article.

If the article material and the gas forming substance are such that the former will absorb the latter, as when iron molds are used with zinc as the gas forming material, the article may be impregnated or covered with the gas forming material in any suitable way, such as by submerging the article in the molten gasifiable metal until the article at its surface has become saturated therewith. The article is then removed from the molten metal and all the surplus free metal brushed from the surfaces, when it is ready for use in making a large number of castings. The gas forming material may be deposited on the article by directing it in a gaseous condition against the article surface where it will congeal in the form of a powder in some instances, or form a smooth surface metallic coating, depending on the temperature of the article. Also the articles may be placed in a metallic gas which will result in surfacing the article with a gasifiable metal. If oxygen is present some of the metal will be oxidized and deposited. The amount of oxide of the metal that will thus be formed will depend upon the amount or concentration of the oxygen. If oxygen, such as atmospheric oxygen, has opportunity to completely burn the heated vapor, then only the oxide will be deposited on the article. The oxide thus deposited may be partially reduced, either by the reducing action of molten iron and carbon of the iron, if the article is to be used for the manipulation of molten iron, or by the carbon deposited as a coating, as when lamp black is used in connection with molds, or by a reducing flame or it may remain and act as a heat insulating neutral coat that will protect the metal of the mold. The protective material may be applied in any suitable way, such as spraying or painting the material on the article.

Articles formed of compositions or mixtures of certain materials may also be treated with protective substances in the same way that the metallic articles described above are treated, and which will coat in the same manner in connection with the articles and the heated metal.

The articles may be formed of a variety of materials. We have, however, found it preferable to use compositions that contain clay as one of the ingredients. To the clay may be added one or more metals which will melt during the calcination of the clay and thus bind the clay. The composition of the article may therefore be made up of a mixture of clay, iron and nickel, or other ma-

terials, if desired. Articles formed of clay and nickel or of clay and iron, we have found, will take up or absorb large quantities of zinc and will deliver it to the surface of the article in the same regulative way that articles formed of iron will control the zinc supply to the surfaces heated by molten metal.

When the article is formed of a composition of one or more materials, such gas forming material or materials should be selected as may be absorbed by one or more of the ingredients of which the mold is composed, if the protective material is to be incorporated within the article as distinct from being applied to the surface thereof. The protective material selected may therefore be such that it will be absorbed by the clay or it may be such that it will form an alloy with or have an affinity for one or more of the metals incorporated in the article, such as the iron of the article. The protection afforded to the article by the gasifiable material prevents the molten metal from attacking and disintegrating the materials of which the article is composed, thus materially adding to the life of the article.

The protective material may be incorporated in an article formed of the composition described above by gasifying the protective material, preferably in a closed receptacle, so as to exclude air and prevent oxidation of the protective material as in the case of zinc, and thus causing absorption of the gas forming material, which, upon chilling, will be deposited as a solid within the body of the article, such as in the clay as well as in the iron of the article. Articles formed of such compositions may also be coated with suitable gas forming substances in the same manner that iron articles may be coated, as described above.

Our invention contemplates the production of articles for treating molten metals having protective material at or near the surface to be brought in contact with the molten metal, that is, the protective material is located where it will have an active protective relation to the article or the molten metal brought in contact therewith, and the word "at" as used in the claims includes broadly at the surface, on the surface, or within material near the surface of the article, but in each case located in a position where it will function in its action, as between the article and the metal manipulated by the article.

Whether the gas producing substance is incorporated in the article or located merely on the surface of the article, the amount of gasification produced by the heat of the molten metal may be regulated by depositing with or upon the gas forming material a heat insulating material, such as lamp

black or metallic oxide that will not chemically react deleteriously on the materials of the article on the gas forming substances or on the metal manipulated by or contained in the article. When lamp black is used it may be deposited on the surface by means of an incomplete combustion flame produced from hydrogen, carbon gas, such as acetylene gas. When the article is coated as distinct from being impregnated with the gas forming substances the heat insulating material may be deposited on the mold over the gas forming substances, or it may be deposited with the gas forming substances. Thus lamp black or graphite may be used to cover the coatings of the metalliferous material or the oxide of its metal, or it may be deposited with the metalliferous material or the oxide of its metal. Since gas forming substances, such as zinc, magnesium, cadmium, etc., or their oxides prevent the adherence of molten metal to metal or of molten metal to calcined clay, ladles, crucibles, troughs, spouts, and other articles or parts of furnaces used in manipulating certain metals, such as iron, brass, etc., while in a molten state, may be treated with the metalliferous substances. This will not only protect the articles from the effect of the molten metal but will also assure free flow and complete delivery of the hot metal manipulated in the use of the article, and will permit the formation of smooth castings.

15 We claim:

1. An iron mold for casting metals having zinc distributed over its matrix surface.
2. A mold for fusible materials having incorporated therein a material gasifiable below the melting point of steel.
3. A metal mold for fusible materials having incorporated therein a metal that will be absorbed by the castings.
4. A metal mold for fusible materials having a material that will melt below the temperature of molten steel incorporated within the surface of the mold.
5. A metal mold for fusible materials having a metal that will melt below the temperature of molten steel incorporated within the surface of the mold.
6. A mold for fusible materials having zinc oxide distributed over its surface.
7. A mold for casting fusible materials having a metal at its matrix surface that will gasify below the melting point of steel.
8. A mold for casting fusible materials having a protective material located within and distributed through the walls of the mold.
9. A container for molten materials having a metal fusible below the temperature of the molten materials incorporated within the inner surface of the wall of the container.

10. A metal mold for casting fusible materials having a metal fusible below the temperature of the fusible materials incorporated within the surface of the matrix.
11. A metal container having a material that will melt below the melting point of steel incorporated within its surface.
12. A container for molten metals having a metal at its inner surface that will gasify below the melting point of steel.
13. An iron container for molten metal, the wall of the container having zinc incorporated therein.
14. A mold for casting metals, the mold having zinc located at the molding surface.
15. A mold for casting metals, the mold having zinc incorporated therein contiguous to the molding surface.
16. A mold containing iron and having zinc incorporated therein.
17. A mold for casting metals, the mold having a metalliferous substance at the surface of the mold that will form a gas below the temperature of molten iron.
18. A metal container for containing molten metals and having a protective material containing zinc located at the inner surface of the container.
19. A metal container for containing molten metals and having a protective material containing zinc oxide located at the inner surface of the container.
20. A metal mold for casting ferrous metals and having a protective material containing zinc located at the surface of the matrix of the mold.
21. A metal mold for casting ferrous metals and having a protective material containing zinc oxide located at the surface of the matrix of the mold.
22. A container for containing molten metals formed of a material containing iron located near the inner surface of the container and having a protective material containing zinc located at the inner surface of the container.
23. A container for containing molten metals formed of a material containing iron located near the inner surface of the container and having a protective material containing oxide of a metal located at the inner surface of the container.
24. A container for containing molten metals formed of a material containing iron located near the inner surface of the container and having a protective material containing zinc oxide located at the inner surface of the container.
25. A ferrous mold for casting ferrous metals, the surface of the matrix coated with zinc.
26. A ferrous mold for casting ferrous metals, the surface of the matrix coated with zinc oxide.
27. A ferrous mold for casting ferrous

metals, the surface of the matrix coated with zinc and zinc oxide.

28. A container for containing molten metal and having a finely divided adhering metallic oxide on the inner surface thereof.

29. A mold for containing molten metal and having a finely divided adhering metal-

lic oxide on the inner surface thereof, the metal of the oxide having a melting point below that of the said molten metal. 10

In testimony whereof, we have hereunto signed our names to this specification.

HUBERT A. MYERS.

ARTEEMES D. STRAW.